

C. BURIAN.

PROCESS FOR CASE HARDENING IRON AND STEEL ARTICLES.

APPLICATION FILED JULY 14, 1913.

1,091,286.

Patented Mar. 24, 1914



Witnesses:

Chas. A. Rose

*Signature*

Inventor  
Carl Burian  
by

*James L. Morris*  
Attorney

# UNITED STATES PATENT OFFICE.

CARL BURIAN, OF BERLIN, GERMANY, ASSIGNOR TO THE FIRM OF GEHRUDER SCHUBERT, OF BERLIN, GERMANY.

## PROCESS FOR CASE-HARDENING IRON AND STEEL ARTICLES.

1,091,286.

Specification of Letters Patent.

Patented Mar. 24, 1914.

Application filed July 14, 1913. Serial No. 779,013.

To all whom it may concern:

Be it known that I, CARL BURIAN, citizen of the Empire of Germany, residing at Berlin, Germany, have invented certain new and useful Improvements in an Improved Process for Case-Hardening Iron and Steel Articles, of which the following is a specification.

My invention relates to an improved process for case-hardening iron and steel articles.

It has already been proposed to harden articles of low-carbon steel by coating them with an adhesive mass containing a fluid or pasty hardening composition and exposing them to the fire in that condition. It has also been proposed to add to the coating mass, saltpeter, common salt, glass and the like, which also serve as a binding medium for the hardening agent and are intended to prevent portions of same from dropping off into the fire. It has, however, been found in practice that satisfactory hardening cannot always be obtained by the aid of the means hitherto proposed, since the binding media used crumble away—especially in an open fire—and drop away, along with the hardening agent, from the surface of the articles to be hardened. According to my present invention, this drawback is intended to be remedied by coating the article with a fluid or pasty hardening composition in the usual way and then surrounding it with a band composed of highly refractory material and coated with a hardening composition on both sides, the article so prepared being then coated with a heat-resisting mass or paste containing powdered fire-resisting materials, such, for example, as asbestos, mica or the like. By means of the band, the hardening composition is reliably retained against the surface to be hardened, no matter whether the hardening is performed in an open fire, in molten salts, a muffle, or in a metal bath.

Referring to the accompanying drawing, which illustrates a practical application of the process, the bolt 1 of iron is wrapped twice at the part 2 to be hardened, with a band 3. This wrapping carries on both sides the hardening powder 4, which has been attached by a binder.

The numeral 5 designates the loam, clay or like material which covers the bolt and its wrapping.

55 The following particulars may serve to

illustrate the carrying out of my process by way of example: The portions of the work that are to be hardened are brushed over with the sticky hardening composition, and the aforesaid band is lapped around the 60 places which have been made sticky, so that the band fits firmly against the work. Such bands are prepared by first dipping a strip in the aforesaid sticky hardening composition and then allowing it to dry after hardening powder has been applied on both 65 sides. The bands can be made of any desired shape and size and of any desired width and thickness, as the particular conditions of the articles to be hardened require. The article surrounded by the band in the manner described above, is then dipped in a liquid heat-resisting mass or paste, to which finely powdered fireproof materials, such as asbestos, mica and the 70 like have been added; or else the article is coated over with such a paste or with loam and is then allowed to dry thoroughly. The articles treated in this manner are warmed up, in any way, to about 400° C., and are 75 then heated to the hardening temperature, for example in a molten salt. When the case-hardening is completed, the articles are freed from their envelop by beating, and are cooled, as usual, in water or oil according to the character desired for them.

I claim:

1. A process for case-hardening iron and steel articles consisting in coating the articles on the places to be hardened with a 90 hardening agent, in surrounding the coated articles by a band containing a hardening agent, in treating the articles so prepared with a heat resisting paste and in heating them to the hardening temperature.

2. A process for case-hardening iron and steel articles consisting in coating the articles on the places to be hardened with a 95 pasty hardening composition, in surrounding the coated articles by a band containing a hardening agent, in treating the articles so prepared with a heat resisting paste and in heating them to the hardening temperature.

3. A process for case hardening iron and steel articles consisting in coating the articles on the places to be hardened with a 105 hardening agent, in surrounding the coated articles by a band of a highly refractory material containing a hardening agent, in treat-

- ing the articles so prepared with a heat resisting paste and in heating them to the hardening temperature.
4. A process for case hardening iron and steel articles consisting in coating the articles on the places to be hardened with a hardening agent, in surrounding the coated articles by a band containing a hardening agent, in treating the articles so prepared with loam and in heating them to the hardening temperature.
5. A process for case-hardening iron and steel articles consisting in coating the articles on the places to be hardened with a heat resisting paste containing powdered fire resisting substances and in heating them to the hardening temperature.
- 10 6. A process for case-hardening iron and steel articles consisting in coating the arti-

cles on the places to be hardened with a hardening agent, in surrounding the coated articles by a band containing a hardening agent, in treating the articles so prepared with loam and in heating them to the hardening temperature.

20

In testimony whereof I have hereunto set my hand in presence of two subscribing witnesses.

CARL BURIAN.

Witnesses:

WOLDEMAR HAUPT,  
HENRY HASPER.